

Aug. 28, 1934.

W. SCHNEIDER

1,971,430

ANTIHALATION LAYER

Filed April 30, 1932



Inventor:  
William Schneider,  
By Attorney  
Philip S. Sophie.

## UNITED STATES PATENT OFFICE

1,971,430

## ANTIHALATION LAYER

Wilhelm Schneider, Dessau in Anhalt, Germany,  
assignor to Agfa Ansco Corporation, Bing-  
hamton, N. Y., a corporation of New York

Application April 30, 1932, Serial No. 608,518  
In Germany May 8, 1931

10 Claims. (Cl. 95—8)

My present invention relates to the manufacture of anti-halation layers for photographic material and more particularly to anti-halation layers which present some advantages when applied to photographic materials destined for the reversal process.

One of its objects is to provide an anti-halation layer which is easily removable in the reversal baths, while the film support is colored with a dye covering the gaps of absorption of the removable anti-halation layer and giving at the same time an agreeable impression to the spectator of the finished material. Further objects will be apparent from the detailed specification following hereafter.

According to this invention the photographic material is provided with an anti-halation layer comprising colloidal silver, that is to say, silver in such a state that the single particles cannot be discerned with the microscope, and a binding agent. Such a layer of colloidal silver has the action of a light filter the spectral permeability of which depends upon the size of the colloidal silver particles. The larger the particles the more the permeability will be shifted from the yellow to the green region of the spectrum. The size of the particles can be influenced by the addition of a suitable electrolyte, such as disodium phosphate, during or after the manufacture of the mixture of colloidal silver and binding agent, the addition of an electrolyte causing an increase in the size of the particles. I prefer to operate in such a manner that the anti-halation layer be permeable to the range from about 550 to 700  $\mu\mu$ . In this case the support is dyed blue or violet, for instance lavender. As suitable dyes I mention light blue (Schultz, Farbstofftabellen 1923, Nr. 521), aniline blue (Schultz, Farbstofftabellen 1913, Nr. 521), violet B (Schultz Farbstofftabellen 1923, Nr. 517). A lavender color is obtainable by mixing a blue dye with rhodamin 3 B (Schultz, Farbstofftabellen 1923, Nr. 574). Preferably a dye is selected which gives an agreeable impression to the spectator. As a binding agent for the colloidal silver layer I prefer gelatin but other binding agents, such as casein or the calcium salt of polyglucuronic acid likewise may be used. The anti-halation layer proper may be arranged between the light-sensitive emulsion layer and the support or it may be applied to the rear side of the support. In the developing process the colloidal silver is dissolved in the reversal bath, for instance, the acid bichromate solution. The dye used for coloring the film is insoluble in the photographic baths.

Instead of the dyes which give an agreeable impression to the spectator of the finished photographic material dyes which do not give such an impression to the spectator likewise may be used, however, in this case the dyes must be removed during the reversal developing process. These dyes may be incorporated in the same layer as the colloidal silver or they may be applied in a separate layer. Suitable dyes are, for instance, those which are described in my copending application Serial Number, 586,966, filed January 15, 1932. In case of employing these dyes preferably an acid permanganate solution is used as reversal developing bath instead of the acid bichromate bath. The gelatin or other binding material containing the dyes may be prepared as described in my said copending application and may then be mixed with the gelatin containing the colloidal silver.

The following examples serve to illustrate the invention:

*Example 1.*—A solution of 25 grams of hydrazine sulfate in 500 grams of water is added to a solution of

1000 grams of water 80

100 grams of silver nitrate

200 grams of ammonia of 30 per cent strength and

190 grams of gelatin

in the course of 1 hour at a temperature of 60° C. 85

Heating is then continued for further 45 minutes. Hereafter the solution is allowed to solidify, cut into small pieces and washed with water for about

1 to 2 hours. After having been molten the product is applied in the usual manner to a support 90

which has been dyed with aniline blue. In case of a support made of nitrocellulose a solution of

5 to 10 grams of dyestuff in 100 parts of a mixture of methanol and alcohol 4:1 is used and in the

case of a support made of acetyl cellulose a solution of 5 to 10 grams of dyestuff in 100 parts of

a mixture of methanol and acetone 4:1 is used for dyeing the support. 95

*Example 2.*—50 per cent of a gelatin containing colloidal silver prepared according to Example 1 100

and 50 per cent of gelatin containing the coupling product of 1,7-aminonaphthol and dianisidine are

mixed and this mixture is applied in known manner as anti-halation layer. The gelatin containing the said coupling product is obtainable as 105

follows. A solution of 50 to 100 parts by weight of gelatin in 800 parts by weight of water is

mixed with 100 parts by weight of  $\frac{1}{10}$  molal solution of 1,7-aminonaphthol and 3 parts by weight of sodium carbonate. This mixture is brought to 110

a temperature of about 25° C. and there are added 100 parts by weight of  $\frac{1}{10}$  molal diazo solution of dianisidine. The resulting mass is allowed to solidify, cut in pieces, washed and molten and 5 is then ready for use.

The accompanying drawing illustrates my invention and is in itself explanatory. I do not intend to limit my invention thereto, other arrangements or combinations of the support, the 10 proper anti-halation layer and the light-sensitive emulsion layer being possible.

My invention is not limited to the foregoing examples or to the specific details given therein. Numerous other embodiments are possible, so, for 15 instance, other dyes than those mentioned may be used, or dyes may be used which are soluble in the alkaline developer. I contemplate as included within my invention all such modifications as fall within the scope of the appended claims.

20 What I claim is:

1. A process for manufacturing anti-halation layers which comprises dissolving silver nitrate in an aqueous solution of a binding agent containing ammonia, precipitating the silver in colloidal form by adding a reducing agent, allowing the solution to solidify, reducing the solidified mass to small pieces, washing the pieces and preparing the anti-halation layer from this product.

25 2. A process for manufacturing anti-halation layers which comprises dissolving 100 parts by weight of silver nitrate in a solution comprising

1000 parts by weight of water

190 parts by weight of gelatin and

30 200 parts by weight of ammonia solution of 30 per cent strength, adding to the said solution 25 parts by weight of hydrazine sulfate dissolved in 500 parts by weight of water in the course of 1 hour at a temperature of 60° C., continuing heating for further 45 minutes, causing then the solution to solidify, reducing the solidified mass to small pieces, washing the pieces for about 1-2 hours and producing the anti-halation layer from the product thus obtained.

35 3. A photographic article comprising a light sensitive emulsion, a support for said emulsion and an anti-halation layer attached to said support comprising colloidal silver and a binding agent.

40 4. A photographic article comprising a light

50

sensitive emulsion, a support for said emulsion and an anti-halation layer attached to said support, said anti-halation layer being permeable to the wave lengths from about 550 to 700  $\mu\mu$  comprising colloidal silver and a binding agent.

80

5. A photographic article comprising a light sensitive emulsion, a support for said emulsion and an anti-halation layer attached to said support, said anti-halation layer being permeable to wave lengths from about 550 to 700  $\mu\mu$  comprising colloidal silver and a binding agent, and said support being colored with a dye covering the gap of absorption of said anti-halation layer.

85

6. A photographic article comprising a light sensitive emulsion, a support for said emulsion and an anti-halation layer attached to said support, said anti-halation layer being permeable to wave lengths from about 50 to 700  $\mu\mu$  comprising colloidal silver and a binding agent, and said support being colored with a dye covering the gap of absorption of said anti-halation layer, and constituting a permanent coloration suitable in projecting the finished film.

90

7. A photographic article comprising a light sensitive emulsion, a support for said emulsion and an anti-halation layer attached to said support, said anti-halation layer being permeable to wave lengths from about 550 to 700  $\mu\mu$  comprising colloidal silver and a binding agent, and said support being dyed with a mixture of light blue 105 and rhodamin.

100

8. A photographic article comprising a light sensitive emulsion, a support for said emulsion and an anti-halation layer attached to said support comprising colloidal silver, a dye soluble in 110 a photographic reversal bath, and a binding agent.

110

9. A photographic article comprising a light sensitive emulsion, a support for said emulsion and an anti-halation layer attached to said support comprising colloidal silver, the coupling 115 product of 1,7-aminonaphthol and dianisidine, and a binding agent.

120

10. A photographic article comprising a light sensitive emulsion, a support for said emulsion and an anti-halation layer attached to said support, said anti-halation layer being permeable to wave lengths from about 550 to 700  $\mu\mu$  comprising colloidal silver and gelatin.

WILHELM SCHNEIDER.

125

55

130

60

135

65

140

70

145

75

150